

Patented July 12, 1927.

1,635,660

# UNITED STATES PATENT OFFICE.

RAY G. COATES, OF PASADENA, CALIFORNIA, ASSIGNOR, BY MESNE ASSIGNMENTS, OF ONE-HALF TO THE ESTATE OF H. G. HAMILTON, DECEASED, LATE OF YOUNGSTOWN, OHIO.

## METHOD OF FINISHING CASTINGS SUCH AS INGOT MOLDS.

No Drawing.

Application filed July 18, 1924. Serial No. 726,756.

The present invention relates broadly to metallurgy and more especially to a method of finishing castings such as ingot molds or the like.

5 Heretofore in the art where large castings are cast in open molds, such as the molds which are used for manufacture of cast iron ingot molds, the upper surface of the metal is usually rough because it is usually in contact with atmosphere only and is not shaped or smoothed by contact with a matrix wall.

10 10 contact with atmosphere only and is not shaped or smoothed by contact with a matrix wall. In such castings, it is customary to smooth the rough portion of the casting by cutting off or cutting away the roughened surface portion. This is especially true in connection with the manufacture of cast iron ingot molds by using the inverted position for casting, such as is disclosed in my Patent

15 No. 1,376,403, patented May 3, 1921.

20 Heretofore in the art, it has been customary to perform the operation of cutting or sawing away the undesirable portion after the mold is completely cooled and has reached atmospheric temperature. When the casting is first shaken out of the sand flask mold, sand tightly adheres to the surface of the casting, but as the casting cools down, the shrinkage causes the mold sand to loosen and therefore when the ingot molds are cut cold, 25 the surface of the ingot is comparatively clean of sand and the mold sand does not interfere with the cutting off operation.

The principal object of the present invention is to reduce the time and expense 30 of the cutting off operation as applied to large castings by performing the cutting operation as soon as the casting has solidified and before it has lost its initial heat after solidification.

40 Another object of the present invention is the method of finishing ingot molds cast in sand molds by cutting the rough portions therefrom after the ingot mold has solidified and before it has lost its initial heat 45 by first removing the mold sand from the surfaces through which the cutting operation extends, and then performing the cutting operation.

Another and more specific object of the 50 present invention is the method of cutting portions from ingot molds cast in sand molds which comprises removing a narrow band of mold sand from around the casting while the casting retains its initial heat and then

cutting the casting on the line of the cleared sand.

Other and further objects of the present invention will be obvious and will in part be pointed out hereinafter in the specification following.

A more specific disclosure of the present invention will now be set forth and it comprises cutting off the undesired portions of a cast iron ingot mold as soon as possible after the ingot mold is shaken from the sand flask and after the cast mold has sufficiently solidified to be safe from bleeding. When this stage of the cast mold is reached the iron is red hot but is comparatively soft and may be cut at a much higher speed and with considerably less energy than is required when the cast mold is completely cooled. A large amount of mold sand adheres to the red hot casting at this stage and this sand has a deleterious effect on cutting tools because of its abrasive action thereon. In carrying out my method as applied to a hollow casting such as an ingot mold, a narrow band of the mold sand is removed from both the inside and outside of the mold and the cutting tool is then operated over and through this narrow band. The removal operation may be done simultaneously with, but slightly in advance of, the entry of the cutting off tool into the work. This prevents any substantial chilling of the metal over the cutting area or zone. The cutting off and the clearing of the sand may be done by any appropriate devices, such as a hot metal saw and an appropriate cleaning device which proceeds the saw.

By the use of the improved method, the sand mold flasks are released for further operations quickly and the cutting operation may proceed with far greater rapidity and with less effort than where the old practice is followed. After the cutting or finishing is completed, the casting with the adhering sand thereon may be annealed in a hot pile or in a special oven according to the practice in the art. The adhering sand greatly retards the cooling of the casting, thus facilitating the annealing.

It is apparent that the herein disclosed method of finishing castings is a very economical one in several respects. The undesirable portions are cut off at a red heat, thus economizing in cutting power.

The heat which may be utilized is the original casting heat and hence the expense of reheating may be eliminated. Injury to the cutting tool by sand is avoided by cleaning the cutting zone, but at the same time the sand is retained on the rest of the casting, thus retarding the cooling of the casting during annealing.

From the foregoing, I desire that it be understood that this method is not limited to cutting away merely the bottom part of ingot mold casting, but is adaptable for use in cutting or finishing either end of such ingot mold, or the like, dependent upon whichever end of the ingot mold contains that portion which requires cutting away or finishing.

Having thus described my invention, what I claim is:

1. The method of finishing large castings cast in sand molds, comprising taking the casting from the flask as soon as the metal in the casting has set, removing the adhering sand throughout a zone where the casting is to be cut, and severing undesirable portions from said casting by cutting through the sand cleaned zone immediately after the removal of the casting from the flask and be-

fore the initial heat of the metal has dissipated sufficiently to cause the casting to completely harden.

2. The method of finishing ingot molds or the like cast in sand molds, which method comprises removing the ingot mold from the flask as soon as the metal has set and sawing away undesired end portions while the ingot mold is retained at red heat by the initial heat of the metal, annealing the ingot mold and utilizing the adhering sand to retard the rate of cooling during annealing.

3. The method of finishing cast iron ingot molds cast in a sand matrix which method comprises removing the ingot mold from the flask as soon as the metal in the ingot mold has solidified, then removing the adhering sand from a portion of the inside wall and the opposite portion of the outside wall of the ingot mold, severing the end from the mold by cutting at right angles to the axis of the ingot mold through the surfaces from which the adhering sand has been removed, annealing the finished ingot mold and utilizing the adhering sand to retard the rate of cooling during annealing.

RAY G. COATES.